

# United States Patent [19]

Iwano et al.

[11] 3,909,267

[45] Sept. 30, 1975

[54] STABILIZATION PROCESS FOR COLOR  
PHOTOGRAPHIC MATERIALS

[75] Inventors: **Haruhiko Iwano; Kazuo Shirasu; Tadao Hatano**, all of Minami-ashigara, Japan

[73] Assignee: **Fuji Photo Film Co., Ltd.**, Minami-ashigara, Japan

[22] Filed: **Dec. 13, 1973**

[21] Appl. No.: **424,253**

[30] Foreign Application Priority Data

Dec. 13, 1972 Japan ..... 47-124915

[52] U.S. Cl. ..... **96/56; 96/22; 96/111**

[51] Int. Cl.<sup>2</sup> ..... **G03C 7/00**

[58] Field of Search ..... 96/56, 111, 22

[56]

References Cited

UNITED STATES PATENTS

|           |         |                   |        |
|-----------|---------|-------------------|--------|
| 2,657,139 | 10/1953 | Bates .....       | 96/56  |
| 3,140,177 | 7/1964  | Welch.....        | 96/56  |
| 3,424,580 | 1/1969  | Wainer .....      | 96/33  |
| 3,582,347 | 6/1971  | Holly et al. .... | 96/111 |
| 3,666,468 | 5/1972  | Amano et al. .... | 96/56  |
| 3,676,136 | 7/1972  | Mowrey .....      | 96/56  |

Primary Examiner—J. Travis Brown

Attorney, Agent, or Firm—Sughrue, Rothwell, Mion, Zinn & Macpeak

[57]

ABSTRACT

The physical properties and storage stability of color photographic papers are improved by processing them in a stabilization bath containing a water-soluble zirconium salt and a polycarboxylic acid.

11 Claims, No Drawings

## STABILIZATION PROCESS FOR COLOR PHOTOGRAPHIC MATERIALS

### BACKGROUND OF THE INVENTION

#### 1. Field of the Invention

The present invention relates to a stabilization process for color photographic materials and, more particularly, it relates to a process for improving the physical properties of color photographic materials and the storage stability of color photographic images.

#### 2. Description of Prior Art

It is known that the stabilization bath used in the processing of photographic light-sensitive materials has a very important relation to the stability of the images of the photographic material and various studies have been made on stabilization. For instance, as disclosed in the specification of U.S. Pat. No. 2,788,274, the fading of color images of color photographic materials can be effectively prevented by processing the color photographic materials with an aqueous solution of a zinc compound. However, this process is not effective for preventing the formation of stains due to the action of light and heat.

Also, it is known to add a polycarboxylic acid to a stabilization bath as described in the specification of British Patent No. 736,881, *The British Journal of Photography*; July 8, 1966, pages 588-589, and *ibid.*; Sept. 27, 1968, pages 838-840. By this process the image stability can be improved with an increase in the content of the polycarboxylic acid but the physical properties of the photographic material are degraded with the increase of the content of the polycarboxylic acid and, hence, the process has a demerit in that it does not satisfy simultaneously improvement in the image stability and the physical properties of photographic materials.

On the other hand, it is known that a stabilization bath containing a water-soluble aluminum salt and a polycarboxylic acid can improve simultaneously the image stability and physical properties of photographic materials as described in U.S. Pat. 3,666,468 but the improvement by the process is not satisfactory.

The reaction of physical properties of photographic materials after processing includes the following various matters.

Photographic papers which have been subjected to photographic processing are usually stored by mounting them on a pasteboard mat or in an album having a transparent film cover or by placing them directly in a bag or box. The temperature and humidity in the storage of the processed photographic papers depend on the season, the climate, and the location but in any case, if the storage conditions are at low temperature and low humidity, physical difficulties such as adhesion or stickiness is less and they increase as the temperature and humidity increases. For instance, when color prints obtained by the known processes as described in the above-mentioned *The British Journal of Photography*; July 8, 1966, pages 588-589, *ibid.*, Sept. 27, 1968, pages 838-840, and the specifications of British Pat. No. 736,881, and U.S. Pat. No. 3,666,468 are preserved under a high-humidity conditions, the following difficulties tend to occur:

1. When the photographs are mounted on both sides of the mats of a usual album, the photographs which are brought into contact stick each other.

2. When the photographs are mounted on a mat of an album having a transparent cover film on the mat, Ne-

ton's rings are formed or dissolved matter in the cover film, such as plasticizers, causes sticking.

3. When the photographs are stacked together in a bag or box, they stick to each other.

4. In any of these cases, the surface of the photographs becomes sticky, fingerprints are left thereon or dust sticks thereto making the images dull.

Also, it is well known that electrostatic charges are frequently formed in an ordinary processing step, in particular the drying step for photographic papers, and if such electrostatic charges are formed on photographic papers, the stacked photographic papers after cutting will be disordered or the photographic papers will stick to each other complicating counting or checking them.

Furthermore, the steps for processing photographic papers having a baryta-coated paper as the support include a drying step using a ferrotype dryer. In particular, in drying color photographic papers using a ferrotype dryer, the hardening bath and stabilization bath becomes frequently questions since they are subjected to various processings before drying. For instance, when the color photographic paper processed in the manner as described in *The British Journal of Photography*, Sept. 27, 1968, pages 838-840 and the specification of British Pat. No. 736,881 is subjected, as it is, to high-temperature high-speed ferrotype drying, the photographic paper sticks to the ferrotype plate. Such inconvenience is considerably improved by using, in drying a rolled photographic paper, the predryer and the re-wetting means as described in "Kodak Products for the Professional", page 6977 (1968) but this attempt has the disadvantage that the aforesaid means additionally is required. Other attempts have been proposed on techniques for polishing the ferrotype plate and on various processing compositions but those attempts have also the defect that they are quite troublesome.

On the other hand, it is known that a photographic material itself or a processing bath gets musty under certain conditions and various attempts have been made for preventing the materials from getting musty. For instance, such attempts are the processes as described in *Photographic Science and Engineering*, 3, 3,132 (1959) and the specification of U.S. Pat. No. 3,093,479.

### SUMMARY OF THE INVENTION

An object of this invention is, therefore, to provide a stabilization process for color photographic materials for improving the physical properties of the color photographic materials.

Another object of this invention is to provide a stabilization process for improving the storage stability of color photographic images.

Still another object of this invention is to provide a processing bath for color photographic materials for improving the above-mentioned physical properties and storage stability, in which the bath itself is also quite stable.

The aforesaid object of this invention can be attained by processing color photographic materials with a processing bath containing a water-soluble zirconium salt and a polycarboxylic acid.

That is to say, the present invention provides a process of processing color photographic materials which comprises processing color photographic materials

with a bath containing a water-soluble zirconium salt and a polycarboxylic acid.

#### DETAILED DESCRIPTION OF THE INVENTION

Suitable water-soluble zirconium salts which can be used in this invention, are zirconium salts such as zirconium sulfate, zirconium nitrate, zirconium chloride, zirconium oxysulfate, zirconium oxynitrate, and zirconium oxychloride. Of these zirconium salts as illustrated above, zirconium oxysulfate is particularly effective. The zirconium salts can be used individually or as a mixture of two or more salts and the amount of the zirconium salt generally used 1 to 20 g/liter, preferably 2 to 6 g/liter.

Also, suitable polycarboxylic acids which can be used in this invention are acids such as oxalic acid, malonic acid, malic acid, tartaric acid, succinic acid, citric acid, glutaric acid, adipic acid, lactic acid, crotonic acid, acetoacetic acid, itaconic acid, diglycolic acid, and citraconic acid and the salts of these acids, such as the alkali metal salts, e.g., the sodium and potassium salts, ammonium salts, etc. Suitable polycarboxylic acids which can be used in this invention are disclosed, for example, in U.S. Pat. Nos. 2,515,121; 2,518,686; 3,140,177; 3,582,332; and 3,676,136. The polycarboxylic acids or the salts thereof can be used individually or as a mixture of them and the amount of the polycarboxylic acid generally used 1 to 15 g/liter, preferably 2 to 10 g/liter.

It is well known that a polycarboxylic acid acts as a buffer for a stabilization bath but the feature of this invention is in the point that an even higher buffer action is obtained using the polycarboxylic acid together with the zirconium salt.

The stabilization bath of this invention is used at a pH of 2.7 to 4.5, preferably 3.3 to 4.0. The pH of the stabilization bath of this invention can be adjusted using an alkali such as sodium hydroxide, sodium metaborate, borax, amine, etc., or an acid such as boric acid, acetic acid, sulfuric acid, etc., as disclosed in U.S. Pat. Nos. 2,515,121; 2,518,686; 3,140,177; 3,582,332, 3,676,136 and 2,647,057.

Another manner of using a zirconium salt which is different from the present invention is in a hardening bath containing a zirconium salt as disclosed in the specification of British Pat. No. 1,271,025. However, although such a known bath may be effective for hardening during processing, the bath is not effective for improving the image stability and the physical properties of photographic materials after processing and hence it is clear that this is different from the process of this invention is effect and the manner of using.

On the other hand, the objects of this invention as described before are not attained by using a bath containing a zirconium salt or a zirconium salt and an aldehyde. In other words, the objects of this invention are attained by processing color photographic papers with a bath containing simultaneously a water-soluble zirconium salt and a polycarboxylic acid or a salt thereof, with the pH of the bath having been adjusted to 2.7 to 4.5, as a final step in the color process for the color photographic papers.

The processing bath of this invention containing the water-soluble zirconium salt and the polycarboxylic acid or a salt thereof can further contain at least one of a compound having an aldehyde group and a compound capable of forming formaldehyde.

Suitable water-soluble compounds having an aldehyde group used in the aforesaid case are compounds represented by the general formula



wherein R represents a hydrogen atom, an alkyl group, an alkenyl group, an aryl group, a carboxyl group, or 10 a heterocyclic ring residue, said R may have been substituted, and when R is a hydrogen atom, n represents an integer and when R is a substituent other than a hydrogen atom, n is 1.

Specific examples of compounds represented by the 15 general formula (I) are formaldehyde, paraformaldehyde, acetaldehyde, aldol, propionaldehyde, acrolein, crotonaldehyde, salicylaldehyde, glyoxylic acid, muconic acid, mucobromic acid, furfural, diglycolaldehyde, etc. Also, precursors of compound of the general 20 formula (I) can be used as the water-soluble compound having an aldehyde group.

Also, as the compound having an aldehyde group, the dialdehyde compounds represented by the general formula (II) can be used.



wherein  $R_1$  represents a divalent aliphatic residue or a 30 divalent aromatic residue, and m is 0 or 1.

Specific examples of compounds represented by the general formula (II) are glyoxal, succinaldehyde, glutaraldehyde,  $\alpha$ -methylglutaraldehyde, cyclopentane-dicarboxyaldehyde and the dialdehydes described in the specification of British Pat. No. 1,102,001, e.g.,



and in the specification of U.S. Pat. No. 3,565,632, e.g.,



Also, precursors of the compound of the general formula (II), such as 2,5-dialkoxytetrahydrofuran as described in the specification of Japanese Pat. publication No. 27,570/1964 can be used as the water-soluble compound having an aldehyde group.

Furthermore, as the compound capable of forming formaldehyde, compounds represented by the following general formula (III) and N-methylol compounds can be effectively used;



wherein R represents an aliphatic group, an aromatic group, or a heterocyclic ring residue.

Examples of compounds represented by the general formula (III) and the N-methylol compounds are N-methylolurea, N,N'-dimethylolurea, N-methylolmethylenebismonoethylurea, N'-methylol-N,N'-dimethylolurea, methylolhydantoin, hydroxydimethyl-

biuret, trihydroxymethylbiuret, 2,2,6,6-tetramethylol-cyclohexanol, methylol dicyandiamide, the compounds described in the specification of British Pat. No. 1,116,944 (such as 3-hydroxy-2,2-dihydroxymethyl-propionic acid), the 2-nitroethanol derivatives described in the specification of British Pat. No. 1,258,359 (such as 2-nitro-2-methyl-1,3-propanediol, and N-hydroxymethylmorpholine).

Suitable examples of aldehydes which can be used in the stabilizing bath are disclosed in U.S. Pat. Nos. 10 2,518,686 and 3,140,177.

The water-soluble aldehyde compound or the compound capable of forming formaldehyde as described above can be used in an amount sufficient to attain the objects of this invention but the amount of the aldehyde compound generally used is about  $1.2 \times 10^{-2}$  to 15  $1.8 \times 10^{-1}$  mol/liter, preferably  $4.2 \times 10^{-2}$  to  $1.1 \times 10^{-1}$  mol/liter and the amount of the compound forming formaldehyde generally used is  $1.0 \times 10^{-2}$  to  $1.7 \times 10^{-1}$ , preferably  $4.1 \times 10^{-2}$  to  $1.2 \times 10^{-1}$  mol/liter. Of 20 the aldehyde compounds described above, in using the dialdehyde compounds better results can be obtained by using it in an amount of  $1.0 \times 10^{-2}$  to  $1.7 \times 10^{-1}$  mol/liter.

On the other hand, a method of improving the stability of a magenta image by processing a photographic material containing a pyrazolone coupler with a stabilization bath containing a polycarboxylic acid and an aldehyde is known as disclosed in the specification U.S. Pat. No. 3,140,177. However, although the method 25 may be excellent in image stability, when the polycarboxylic acid and the aldehyde are used in the amounts disclosed in the specification of this U.S. patent, the photographic materials thus processed are greatly reduced in physical properties. In particular, when the amount of the aldehyde is increased, the physical properties of the processed photographic material are greatly degraded and the use of these compounds is unpleasant because of their irritative smell. Further stains 30 are readily formed depending on the storage conditions. Hence, the objects of this invention can not be attained using such a known method.

The processing bath of this invention containing the water-soluble zirconium salt and the polycarboxylic acid or a salt thereof can further contain a water-soluble organic acid such as benzoic acid or an alkali metal salt of benzoic acid. A suitable level of use ranges from about 0.01 to 10 g/l, preferably 0.1 to 1 g/l, for the 35 benzoic acid or its alkali metal salt.

It is desired that the stabilization bath of this invention be used fundamentally after finishing the development steps of color photographic materials, that is to say, after finishing the development, bleaching, and fixing. After processing with the stabilization bath of this 40 invention, the photographic material can be rinsed.

The development steps for color photographic materials which are employed prior to the use of the stabilization bath of this invention can be conventional color processes for color photographic materials as disclosed in U.S. Pat. Nos. 2,515,121; 2,518,686; 2,647,057; 45 3,140,177; 3,582,322 and 3,676,136. The steps include basically the steps of development, bleaching, and fixing as described in, e.g., the publications as described above. Of course, other embodiments of development steps including a blix step or a stopfix step can be employed. Also, any of these steps in the development can be followed by a wash step or another step.

The stabilization process of this invention can be applied to any color photographic materials but it is preferably applied to color photographic paper which have photographic emulsions containing at least one 4-equivalent or 2-equivalent coupler.

Examples of 4-equivalent couplers are shown below:

Namely, the pyrazolone couplers giving a magenta dye represented by the following general formula are particularly useful.



wherein R<sub>3</sub> represents a substituted or unsubstituted alkyl group, a substituted or unsubstituted aryl group, or a substituted or unsubstituted heterocyclic group and R<sub>4</sub> represents an alkyl group, a carbamyl group, an amino group, or an amide group.

Specific examples of the 4-equivalent couplers represented by the above formula are:

1-p-sec-amylphenyl-3-n-amyl-5-pyrazolone,  
2-cyanoacetyl-5-(p-sec-amylbenzoylamino)cumalone,  
2-cyanoacetylcumarone-5-(N-n-amyl-p-t-amylsulfoanilide),  
2-cyanoacetylcumarone-5-sulfon-N-n-butylanilide,  
1-p-laurylphenyl-3-methyl-5-pyrazolone,  
1-β-naphthyl-3-amyl-5-pyrazolone-1-p-nitrophenyl-3-n-amyl-5-pyrazolone,  
1-phenyl-3-acetylamino-5-pyrazolone,  
1-phenyl-3-n-vareamino-5-pyrazolone,  
1-phenyl-3-chloroacetylamino-5-pyrazolone,  
1-phenyl-3-(m-aminobenzoyl)amino-5-pyrazolone,  
1-p-phenoxyphenyl-3-(p-t-amylxybenzoyl)amino-5-pyrazolone,  
1-(2',4',6'-trichlorophenyl)-3-benzamido-5-pyrazolone,  
1-(2',4'-dichlorophenyl)-3-[3''(2''',4'''-di-t-amyloxyacetamido)benzamido]-5-pyrazolone, and  
1-(2,4-dimethyl-6-chlorophenyl)-3-[3''-(2''',4'''-di-t-amyloxyacetamido)benzimido]-5-pyrazolone.

Suitable examples of pyrazolones which are suitable are disclosed, for example, in U.S. Pat. No. 3,582,322.

Also, the 4-equivalent couplers as disclosed in the specifications of U.S. Pat. No. 3,558,319, British Pat. No. 1,142,553, U.S. Pat. No. 3,337,344 and Japanese Pat. publication No. 20,636/1970 can be used for the color photographic papers stabilized by the process of this invention.

Furthermore, the 4-equivalent couplers giving benzoylacetanilide type yellow dyes or pivaloylacetanilide type yellow dyes are described in the specifications of British Pat. No. 1,113,038; U.S. Pat. No. 3,551,156; U.S. Pat. No. 3,337,344; Japanese Pat. publication No. 19,956/1970; and U.S. Pat. application, Ser. No. 319,806, filed Dec. 29, 1972. Specific examples of the 4-equivalent couplers are:

α-{3-[α-(m-pentadecylphenoxy)butylamido]benzoyl}-2-chloroacetoanilide,

$\alpha$ -{3-[ $\alpha$ -(2,4-di-t-  
amylphenoxy)butylamido]benzoyl}-2-  
methoxyacetanilide,  
 $\alpha$ -{3[ $\alpha$ -(2,4-di-t-amylphenoxy)butylamido]benz-  
oyl}-2-chloroacetanilide,  
2-chloro-3'-(2,4-di-t-amylphenoxy)butylamido]ben-  
zoylacetanilide,  
 $\alpha$ -{3-[ $\alpha$ -(2,4-di-t-amylphenoxy)acetamido]benzoyl}  
benzoylacetanilide, and  
 $\alpha$ -pivalyl-2,5-dichloro-4-[N'-(n-octadecyl)-N-  
methylsulfamyl]-acetanilide.

The 2-equivalent couplers as disclosed in the specifications of U.S. Pat. No. 3,582,322 can be used as couplers for color photographic papers processed by the process of this invention. Also, the phenolic couplers giving cyan dyes as disclosed in the specifications of U.S. Pat. No. 2,423,730 and U.S. Pat. No. 2,801,171 can be effectively used.

The color photographic emulsions for the color photographic materials processed by the process of this invention are those prepared by dispersing a silver halide such as silver bromide, silver iodobromide, silver chloride, silver chlorobromide, silver chloroiodobromide, etc., in a natural or synthetic water-soluble polymer such as gelatin, gelatin derivative (e.g., phthalated gelatin, malonated gelatin, etc.,), colloidal albumin, cellulose derivatives, etc., for example, as disclosed in U.S. Pat. No. 3,582,322.

These silver halide photographic emulsions can contain, in addition to the aforesaid couplers, conventional additives well known in the photographic art, such as dye sensitizers, antifoggants, stabilizers, hardening agents, coating aids, etc., as disclosed in U.S. Pat. No. 3,582,322.

The silver halide emulsion as described above is coated on conventional support such as a baryta-coated paper, a polymer-coated paper such as polyolefin coated paper (as disclosed in, e.g., the specifications of Japanese Pat. publication No. 19,164/1968 and British Pat. Nos. 1,314,196 and 1,134,197), and a so-called synthetic paper prepared by making opaque a transparent film of a polymer such as polyolefin, cellulose derivative, etc. Furthermore, when the process of this invention is applied to, in particular, color photographic papers, excellent advantages are obtained.

By the process of this invention the following excellent results are obtained.

1. When photographs processed by the process of this invention are stored in an album for a long period of time under various conditions, neither adhesion nor stickiness is observed.

2. The generation of static charges caused by the friction of the photographs with rollers which are brought into contact with the photographs during the processing and drying steps or with the ferrotype plate is greatly reduced.

3. Images having excellent stability to light are obtained.

4. When the photographs are stored for a long period of time without exposure to light, the stability of the images of the photographs is not degraded.

Moreover, when a baryta-coated paper is used as the support for the photographic paper, the following specific effects are obtained.

1. At ferrotype drying, the photographs do not stick to the ferrotype plate.

2. A predryer required in ferrotype drying in the conventional case becomes unnecessary.

Also, the stabilization bath used in this invention has the following advantages:

1. The stabilization bath does not get musty.
  2. The stabilization bath has a higher buffer action.
- An extremely important advantage of the color photographic paper processed by the stabilization process of this invention is that the photographic paper shows excellent physical properties when the photograph is stored under various conditions and additionally photographs processed by the stabilization process of this invention have stable images as described above is also an excellent advantage of this invention. That is to say, according to the process of this invention, a color photograph having not only a stable magenta color image but also cyan and yellow color images is obtained. Also, when the photographic papers are preserved under various conditions, less formation of stains is observed.
- 20 The image stability of the photograph processed by the stabilization process of this invention is particularly excellent when the photograph is exposed to high-temperature and high-humidity conditions and also to light. The effects or advantages of this invention are confirmed by referring to the method of *Photographic Science and Engineering*; 11, (5), 295-305 (1967).

Also, by the process of this invention, electrostatic charges are formed on the photographic paper to a lesser extent and thus the occurrence of difficulties caused by the formation of static charges can be prevented.

By processing a color photographic paper after color developing, stop-fixing, washing, blixing, washing, bleaching, and washing the color photographic paper in the stabilization bath of this invention, the photographic paper thus processed can be subjected to high-temperature high-speed ferrotype drying directly and without the necessity of predrying. Furthermore, the drying speed of the color photographic paper processed by the process of this invention is higher than that with pretype-drying a photographic paper processed by the aforesaid known development process and dried in a predrying step. Moreover, the color photographic paper thus dried after processing by the process of this invention has superior gloss to the conventionally processed paper. Also, while electrostatic charges are formed even if the color photographic paper processed by the known development processing is dried by ferrotype drying at a low speed, almost no electrostatic charges are formed in drying the color photographic paper processed by the process of this invention.

Still further, because the stabilization bath used in this invention has sufficiently high buffer capacity, satisfactory results can be obtained by conducting the process in any vessel such as a tank, vat, drum, etc. The stabilization bath of this invention is particularly suitable for the continuous processing of a large amount of photographic papers.

Then, the effects of improving the physical properties of color photographic papers, the image stability, and of preventing the stabilization bath from getting musty in using the stabilization process of this invention are shown by the following specific examples although the invention is not limited to these examples by any means. Furthermore, from the examples, it will also become apparent that the objects of this invention are not

attained by using the polycarboxylic acid or a salt thereof and the water-soluble zirconium salt individually or by using the zirconium salt together with an aldehyde compound.

## EXAMPLE 1

| Color Developer                                                     | pH | 10.6   |
|---------------------------------------------------------------------|----|--------|
| Sodium Metaborate                                                   |    | 25.0g  |
| Sodium Sulfite                                                      |    | 2.0g   |
| Hydroxylamine (sulfate)                                             |    | 2.0g   |
| Potassium Bromide                                                   |    | 0.5g   |
| 6-Nitrobenzimidazole (nitrate)                                      |    | 0.02g  |
| Sodium Hydroxide                                                    |    | 4.0g   |
| Benzyl Alcohol                                                      |    | 15.8g  |
| Diethylene Glycol                                                   |    | 20.0ml |
| N-Ethyl-N-β-(methanesulfoneamidoethyl)-p-phenylenediamine (sulfate) |    | 8.0g   |
| Water to make                                                       |    | 11     |
| Stop-fix Solution                                                   | pH | 4.5    |
| Ammonium Thiosulfate                                                |    | 120.0g |
| Sodium Pyrosulfite                                                  |    | 20.0g  |
| Glacial Acetic Acid                                                 |    | 10.0g  |
| Water to make                                                       |    | 11     |
| Bleach Solution                                                     | pH | 7.2    |
| Potassium Nitrate                                                   |    | 25.0g  |
| Potassium Ferricyanide                                              |    | 20.0g  |
| Potassium Bromide                                                   |    | 8.0g   |
| Boric Acid                                                          |    | 5.0g   |
| Borax                                                               |    | 2.5g   |
| Water to make                                                       |    | 11     |
| Hardening-fix Solution                                              | pH | 9.5    |
| Ammonium Thiosulfate                                                |    | 120.0g |
| Sodium Sulfite                                                      |    | 5.0g   |
| Boric Acid                                                          |    | 2.5g   |
| Formalin (35-40%)                                                   |    | 40.0ml |
| Water to make                                                       |    | 11     |

A color photographic paper was prepared by applying to a polyethylene-coated paper a silver bromide emulsion containing a yellow coupler emulsified dispersion, a silver chloride emulsion (silver chloride 70 mol percent) containing a magenta coupler emulsified dispersion, a silver chlorobromide emulsion (silver chloride 70 mol percent) containing a cyan coupler emulsified dispersion, and then a gelatin solution containing a ultraviolet absorbent. The coupler emulsified dispersion used in the preparation of the color photographic paper was prepared by dissolving each coupler in a mixture of dibutyl phthalate and tricresyl phosphate and then dispersing the solution in a gelatin solution in an o/w type using sorbitan monolaurate, Turkey oil, and sodium dodecylbenzenesulfonate as an emulsifying dispersing agent. As the couplers, 1-(2',4',6'-trichlorophenyl)-3-[3''-(2'',4''-di-t-  
amylphenoxyacetamido)benzamido]-5-pyrazolone, 2-(2,4-di-t-amylphenoxyacetamido)-4,6-dichloro-5-methylphenol, and  $\alpha$ -(2-methylbenzoyl)-aceto-(2-chloro-5'-dodecoxy carbonyl) anilide were used. Also, as the ultraviolet absorbent, the compound described in the specification of Japanese Pat. publication No. 9586/1970 was used. In the emulsion, 2,4-dichloro-6-hydroxy-1,3,5-triazine-sodium salt was used.

The color photographic paper thus prepared was exposed using a color printer and then subjected to the following color development at temperatures lower than 30.0°C.

|                   |   |           |
|-------------------|---|-----------|
| Color Development | : | 7 minutes |
| Stop-fixing       | : | 2 minutes |
| Washing           | : | 2 minutes |
| Bleaching         | : | 2 minutes |
| Washing           | : | 2 minutes |
| Hardening-fix     | : | 2 minutes |
| Washing           | : | 4 minutes |

10. Thereafter, the color photographic paper thus processed was further processed in one of the processing solutions A-F shown in the following table.

| Compound            | A    | B    | C    | D    | E     | F     |
|---------------------|------|------|------|------|-------|-------|
| Zirconium Oxsulfate | 4.0g | 4.0g | 4.0g | 4.0g | —     | —     |
| Citric Acid         | 3.5g | 7.0g | —    | —    | 3.5g  | 10.0g |
| Tartaric Acid       | —    | —    | 5.0g | —    | —     | 20.0g |
| Potassium Alum      | —    | —    | —    | —    | 20.0g | —     |
| Sodium Metaborate   | —    | —    | —    | —    | —     | 20.0g |
| Zinc Sulfate        | —    | —    | —    | —    | —     | 10.0g |
| Water to make       | 11   | 11   | 11   | 11   | 11    | 11    |
| pH                  | 3.5  | 3.5  | 3.5  | 3.5  | 3.5   | 3.5   |

The adjustment of the pH was conducted using sodium hydroxide.

After the processing, the image stability was evaluated using the following conditions.

30. That is to say, the fading percentage of the portion having a density of 1.0 and an increased yellow stain density ( $\Delta D_y - 1$ ) of the color photographic paper when it was stored for 14 days in the dark at 37.8°C and a relative humidity of 90% were measured. The results obtained are shown in the following table.

| Processing Bath | Yellow Color Image | Magenta Color Image | Cyan Color Image | $\Delta D_y - 1$ |
|-----------------|--------------------|---------------------|------------------|------------------|
| A               | 6%                 | 3%                  | 5%               | +0.03            |
| B               | 5%                 | 3%                  | 6%               | +0.03            |
| C               | 7%                 | 3%                  | 5%               | +0.03            |
| D               | 16%                | 3%                  | 10%              | +0.25            |
| E               | 20%                | 3%                  | 5%               | +0.05            |
| F               | 15%                | 3%                  | 15%              | +0.20            |

Also, the fading percentage of the portion of density 1.0 and the increased yellow stain density ( $\Delta D_y - 2$ ) 50 when the color photographic paper was preserved for 14 days at 60°C and a relative humidity of 70% were measured. The results obtained are shown in the following table.

| Processing Bath | Yellow Color Image | Magenta Color Image | Cyan Color Image | $\Delta D_y - 2$ |
|-----------------|--------------------|---------------------|------------------|------------------|
| A               | 4%                 | 2%                  | 8%               | +0.02            |
| B               | 4%                 | 2%                  | 7%               | +0.02            |
| C               | 4%                 | 2%                  | 8%               | +0.02            |
| D               | 8%                 | 2%                  | 20%              | +0.20            |
| E               | 5%                 | 2%                  | 10%              | +0.04            |
| F               | 9%                 | 2%                  | 23%              | +0.18            |

65. As is clear from the above results shown in the tables, the stabilization baths of this invention (A-C) was superior in image stability to the known stabilization

baths (D-F). Also, when the color photographic papers thus processed were preserved for 7 days at 76.7°C (the same condition as the drying step), the color photographic papers processed with the stabilization baths of this invention showed less in fading of the cyan color image and less increase in yellow stains as compared with the color photographic papers processed in the known stabilization baths. Furthermore, when the color photographic papers processed were exposed to an xenon lamp or a ultraviolet lamp, the increase in yellow stains was less in the processing with the stabilization baths of this invention as compared with the processing with the known stabilization baths.

Then, color photographic papers were prepared using baryta-coated paper as the support in place of the polyethylene-coated paper using the same manner as described above. After finishing the above-stated processings, the color photographic papers were directly subjected to ferrototype drying at 80°C without applying predrying. The time required for finishing the drying procedure in this case is shown in the following table. The ferrototype dryer MR-3D made by Japo K. K. was used in this step.

| Bath        | A   | B   | C   | D   | E | F  |
|-------------|-----|-----|-----|-----|---|----|
| Time (min.) | 2.5 | 2.5 | 2.5 | 2.5 | 3 | 10 |

As is clear from the above results, the drying period required for drying the photographic papers processed with the stabilization baths A-C was almost same as that in the case of the processing with the known stabilization bath E and was shorter than that in the processing with the known stabilization bath F. Also, the period of time was same as that of the processing with the stabilization bath containing zirconium oxysulfate alone.

Then, the electrostatic charges formed on the photographic papers when they were dried by ferrototype drying were measured. The results obtained are shown in the following table. The electrostatic meter Statiron-M made by Shishida Shokai K. K. was used.

| Drying period | A     | B     | C     | D     | E     | F             |
|---------------|-------|-------|-------|-------|-------|---------------|
| 3 min.        | 0.1kv | 0.1kv | 0.1kv | 0.1kv | 0.2kv | not separated |
| 10 min.       | 0.1kv | 0.1kv | 0.1kv | 0.1kv | 0.1kv | 6.0kv         |

As is clear from the results in the above table, the amount of electrostatic charges formed in the processing with the stabilization baths (A-C) of this invention was almost same as or less than that of the processing with the known stabilization baths. Also, the amount was the same as that of the processing with the bath containing zirconium oxysulfate alone.

Furthermore, the samples thus dried were humidified for one day at a relative humidity of 90% and after stacking the samples so that the emulsion layers contacted each other and placing a load of 1 kg/12cm × 8.3cm<sup>2</sup> on the piled samples, the samples were preserved for one day in that condition. In this case, the emulsion layers of the samples processed with the

known stabilization bath F stuck to each other but no such phenomenon was observed in the other samples. The test corresponds to the preserving of color prints in an album for a long period of time, in particular, under high humidity conditions.

Also, the samples processed with the known stabilization bath F became sticky and it was easy to leave fingerprints on the samples but no such difficulties were encountered with the other samples.

From all of the results described above, it is clear that the color photographic paper processed by the stabilization bath of this invention after development showed excellent image stability and physical properties.

## EXAMPLE 2

The color photographic paper prepared in the same manner as described in Example 1 was processed in a color developer having the same composition as described in Example 1 for 3 minutes and 30 seconds at 31°C and then processed in the blix bath having the following composition for 1 minute and 30 seconds:

| Blix Bath Composition                    |        |
|------------------------------------------|--------|
| Sodium Ferric Ethylenediamine            | 50 g   |
| Tetraacetic Acid                         |        |
| Ethylenediamine Tetraacetic Acid,        | 4.8 g  |
| Tetrasodium Salt                         |        |
| Sodium Sulfite                           | 15 g   |
| Ammonium Thiosulfate (60% aqueous soln.) | 150 ml |
| Ammonium Rhodanide                       | 15 g   |
| Water to make                            | 1 l    |

The color photographic film was washed for 2 minutes and then processed in a stabilization bath having the following composition:

| Stabilization Bath                            |      |
|-----------------------------------------------|------|
| Zirconium Oxysulfate                          | 4.0g |
| Benzoic Acid                                  | 0.5g |
| Citric Acid                                   | 3.5g |
| Additive<br>(as shown in the following table) |      |
| Water to make                                 | 1 l  |

| 55 | Bath                    | Additive | Amount |
|----|-------------------------|----------|--------|
| G  | Formaldehyde            | 5.0g/l   |        |
| H  | Acetaldehyde            | 1.5g/l   |        |
| I  | 4-Hydroxybenzaldehyde   | 4.0g/l   |        |
| J  | Succinaldehyde          | 2.9g/l   |        |
| K  | Glyoxal                 | 2.0g/l   |        |
| L  | Acrolein                | 1.9g/l   |        |
| M  | Crotonaldehyde          | 2.3g/l   |        |
| N  | N,N'-Dimethylolurea     | 4.0g/l   |        |
| O  | Methylol diethanolamine | 4.5g/l   |        |
| P  | Methylothiadantoin      | 4.3g/l   |        |

60 After the procedures were finished, the samples were stored in the dark for 14 days at 37.8°C and a relative humidity of 90%, for 14 days at 60°C and a relative hu-

midity of 70%, or for 7 days at 76.7°C or were exposed to a fluorescent lamp or a xenon lamp. The image stability in these cases was almost same as that in the processing with the stabilization bath A in Example 1. On the other hand, the period of time required for finishing the drying step, the degree of formation of electrostatic charges, and the sticking state under the condition of a relative humidity of 90% were almost the same as the physical properties in the case of processing with the stabilization bath A in Example 1.

Then the stabilization baths G-P of this invention were stored for about 10 weeks, the baths did not get musty while when the known bath E (Example 1) was stored under the same conditions for 2 weeks, a black substance emitting a putrid smell was formed.

#### REFERENCE EXAMPLE

A color photographic paper prepared in the same manner as described in Example 1 was processed in a solution having the following composition for 80 seconds at 38°C.

|                     |     |    |
|---------------------|-----|----|
| Sodium Sulfate      | 150 | g  |
| Formaldehyde        | 10  | g  |
| Glacial Acetic Acid | 1.7 | ml |
| Sodium Bromide      | 2.0 | g  |
| Succinaldehyde      | 1.0 | g  |
| Water to make       | 1   | 1  |

Then, the color paper was processed in a hydroxylamine bath as described in the specification of U.S. Pat. No. 3,168,400 for 40 seconds.

Thereafter, after processing the color paper with the color developer as shown in Example 1 for 7 minutes at 30°C, the color paper was processed in the following stop-fix bath for 2 minutes.

#### Stop-fix Bath

|                                             |       |   |
|---------------------------------------------|-------|---|
| Ammonium Thiosulfate<br>(58% aqueous soln.) | 215   | g |
| Sodium Sulfite                              | 11.2  | g |
| Glacial Acetic Acid                         | 20.0  | g |
| Sodium Hydroxide                            | 9.0   | g |
| Zirconium Oxsulfate                         | 2.12  | g |
| Aluminum Sulfate                            | 34.06 | g |
| Water to make                               | 1     | 1 |

Then, the color paper was washed for 2 minutes, processed for 2 minutes in a bleach bath having the same composition as described in Example 1, washed for 2 minutes, processed for 4 minutes in a hardening-fix bath having the same composition as described in Example 1, and then washed for 4 minutes.

After drying, the image stability of the color paper was tested as described in Example 1, the results of which showed that the image stability was almost the same as that obtained in omitting the processing with the stabilization bath in Example 1. Also, the various physical properties of the color paper were almost the same as those of the sample which was not processed with the stabilization bath in Example 1. From the above results, it is clear that a stabilization bath containing a water-soluble zirconium salt becomes effective when it is used together with a polycarboxylic acid in accordance with this invention.

While the invention has been described in detail and with reference to specific embodiments thereof, it will be apparent to one skilled in the art that various changes and modifications can be made therein without departing from the spirit and scope thereof.

What is claimed is:

1. A stabilization process for a color photographic material having silver halide emulsion layers containing color couplers which react with an oxidation product 10 of a color developer to form color images which comprises processing said color photographic material, after developing and bleaching, with a bath having a pH of 2.7 to 4.5 containing (1) a water-soluble zirconium salt and (2) a polycarboxylic acid or a salt thereof, said 15 stabilization process being the final step in a color development process except for rinsing.

2. A stabilization process for a color photographic paper having silver halide emulsion layers containing color couplers which react with an oxidation product 20 of a color developer to form color images, which process comprises processing said color photographic paper, after developing and bleaching, with a bath having a pH of 2.7 to 4.5 containing a water-soluble zirconium salt and a polycarboxylic acid or a salt thereof, said stabilization process being the final step in color development process except for rinsing.

3. The stabilization process for a color photographic paper as set forth in claim 2, in which said bath contains  $1.2 \times 10^{-2}$  to  $1.8 \times 10^{-1}$  mol/liter of a water-soluble compound having an aldehyde group or  $1.0 \times 10^{-2}$  to  $1.7 \times 10^{-1}$  mol/liter of a water-soluble compound capable of forming formaldehyde, said water-soluble compound having an aldehyde group being selected from the group consisting of a monoaldehyde 35 compound represented by the formula



- 40 wherein R represents a hydrogen atom, an alkyl group, an alkenyl group, an aryl group, a carboxyl group, or a heterocyclic ring residue, wherein said R may be a substituted group, when R is a hydrogen atom n is an integer, and when R is a substituent other than a hydrogen atom n is 1 and a dialdehyde compound represented by the formula



- 45 wherein R<sub>1</sub> represents a divalent aliphatic residue, or a divalent aromatic residue, and m is 0 or 1, said water-soluble compound having a group capable of forming formaldehyde being a compound represented by the formula



- 50 wherein R<sub>2</sub> represents an aliphatic residue, an aromatic residue, or a heterocyclic ring residue.

4. The stabilization process for a color photographic paper as set forth in claim 3, in which the amount of said water-soluble dialdehyde compound is  $1.0 \times 10^{-2}$  to  $1.7 \times 10^{-1}$  mol/l.

5. The stabilization process for a color photographic paper as set forth in claim 2, in which said polycarboxylic acid is oxalic acid, malonic acid, malic acid, tartaric acid, succinic acid, citric acid, glutaric acid, adipic acid, lactic acid, crotonic acid, aconitic acid, itaconic acid, diglycolic acid, citraconic acid, an alkali metal salt of said acid, or an ammonium salt of said acid.

6. The stabilization process for a color photographic paper as set forth in claim 5, in which the amount of the polycarboxylic acid is 1 to 15 g/l.

7. The stabilization process for a color photographic paper as set forth in claim 2, in which said water-soluble zirconium salt is zirconium sulfate, zirconium nitrate, zirconium chloride, zirconium oxysulfate, zirconium oxynitrate, or zirconium oxychloride.

8. The stabilization process for a color photographic paper as set forth in claim 7, in which the amount of 10 said water-soluble zirconium salt is 1 to 20 g/l.

9. The stabilization process for a color photographic paper as set forth in claim 2, in which said stabilization bath contains benzoic acid or an alkali metal salt.

10. A stabilization bath for a color photographic 15 paper containing a water-soluble zirconium salt, a polycarboxylic acid, and at least one of a water-soluble compound having an aldehyde group and a water-soluble compound having a group capable of forming formaldehyde.

11. The stabilization bath of claim 10 wherein the bath has a pH of 2.7 to 4.5, the water-soluble compound having an aldehyde group is present in the amount of  $1.2 \times 10^{-2}$  to  $1.8 \times 10^{-1}$  mol/liter, the water-soluble compound having a group capable of forming 25

formaldehyde is present in an amount of  $1.0 \times 10^{-2}$  to  $1.7 \times 10^{-1}$  mol/liter, said water-soluble compound having an aldehyde group is selected from the group consisting of a monoaldehyde compound represented by the formula



wherein R represents a hydrogen atom, an alkyl group, an alkenyl group, an aryl group, a carboxyl group, or a heterocyclic ring residue, wherein said R may be a substituted group, when R is a hydrogen atom n is an integer, and when R is a substituent other than a hydrogen atom n is 1 and a dialdehyde compound represented by the formula



wherein R<sub>1</sub> represents a divalent aliphatic residue, or a divalent aromatic residue, and m is 0 or 1, said water-soluble compound having a group capable of forming 20 formaldehyde is represented by the formula



wherein R<sub>2</sub> represents an aliphatic residue, an aromatic residue, or a heterocyclic ring residue.

\* \* \* \* \*

30

35

40

45

50

55

60

65